

Oct. 25, 1927.

1,646,907

E. FREUND

ART OF PRODUCING ORNAMENTAL EFFECTS ON WOOD, GLASS, ETC

Filed Aug. 3, 1926



INVENTOR  
*Edward Freund*  
BY  
*J. H. M. J.*  
ATTORNEY

Patented Oct. 25, 1927.

1,646,907

# UNITED STATES PATENT OFFICE.

EDWARD FREUND, OF LONG BEACH, NEW YORK.

## ART OF PRODUCING ORNAMENTAL EFFECTS ON WOOD, GLASS, ETC.

Application filed August 3, 1926. Serial No. 126,906.

My invention relates to a method of ornamenting wood for use as panels in cabinet work, furniture, wall decorations, etc., and the object of my invention is to produce effects having the appearance of marquetry work. By the use of my invention various effects may be produced having exceedingly close resemblance to actual inlaid pieces, but at greatly reduced cost and saving of time, and in many respects far better effects may be obtained by the use of my invention for the reason that by the employment of colors applied by a brush or otherwise very fine lines may be shown which would not be capable of production in actual inlaid work.

I am aware that heretofore attempts have been made to imitate marquetry work and grain effects in wood by paints or colors and partly removing the paint to produce the desired effects, but the methods heretofore proposed have not been satisfactory for various reasons which my invention is designed to overcome.

In carrying my invention into effect in producing plain designs, I first apply to the wood a ground coat of oil stain or paint of the desired color and allow same to dry to the point where it will not readily rub off and permit handling, or it might be allowed to dry and harden. I then apply to the painted surface over the entire area of the design to be produced, a solution containing an oil which will attack the paint and render it soft so that it may be readily removed by rubbing with a piece of cloth or other absorbent material. After the softened paint is removed the design will appear in the form of a silhouette showing in the natural wood and the surrounding area showing the grain through the oil stain or paint. The work may be left in this form and finished with wax finish or a coating of varnish may be applied and left as a glaze coat, or the varnish coating may be rubbed down in the usual manner and one or more coats of varnish applied as usual in finishing furniture or other wood work. When the design is to be of different character or more elaborate in detail, the silhouette is treated by outlining or tracing the border lines in any desired color, preferably in black with india ink; or the design may be fully detailed in the same manner, and when this work is thoroughly dry, the finishing coats may be applied as above stated. Or, when desired, the design may be further treated by applying appropriate colors, either oil or water colors, but preferably the latter, and then finished as above stated.

My invention is illustrated in the accompanying drawing, in which the figure illustrates the several stages of my method as above outlined. The illustration of the several steps in the one figure is done for the purpose of avoiding duplication of the design in illustrating the successive steps of the method.

Referring to the drawing, 1 indicates a board or panel which may be used for any desired purpose such as a panel in a cabinet or other piece of furniture, or as a panel in wall or ceiling decoration, and as will be understood may be of any kind of wood, solid or veneered. 2 indicates one or more ground coats of oil stain or paint of any desired color, and which may be thin or heavy so as to show or cover the grain of the wood, or of a color or material to bring out the characteristics of woods such as mahogany, cherry, birch, oak, etc. This ground coat 2 is applied over the entire surface of the panel 1, and allowed to dry, preferably hard, that is, so that the coating will not rub off or show the effects of rubbing with a cloth or other absorbent material. I then apply over the area of the design, preferably with a fine brush, a solution containing a non-drying oil which softens the oil stain or paint, and which solution will not flow or penetrate the paint beyond the points where applied with the brush. A sufficient interval of time is allowed for the solution to thoroughly soften the paint, the time depending upon the degree of hardness and thickness of the coating. When sufficiently soft, the paint may be readily removed by wiping with cloth or cotton, and owing to the nature of the solution, the removal will be clean and allow the grain of the wood to show clearly in the silhouette as indicated at 3 in the upper half of the illustration; the clear white of the drawing indicating the bare wood or grain. I have found that by the use of my solution the outline of the design, when the paint is removed, appears in clear, sharp, distinct lines showing that the solution does not flow or penetrate the paint beyond the line of application with the brush.

As above stated, the design for some purposes may be left as shown in the upper half of the drawing, or it may be changed or

elaborated to a greater or lesser extent as shown in the lower half of the drawing. This is done by applying colors by means of a brush, pen or other implement. Thus in the lower half of the illustration the flower design is completed by outlining and shading the petals and stamens of the flowers; the blades of the leaves are outlined and shaded, and the veins shown, and the main stem is outlined and shaded. All of this treatment may be in colors, and preferably the outlining is in black with india ink for the purpose of imparting the appearance of inlaid work, and the leaves and flowers may be tinted with appropriate colors. A border effect 4 may be produced in various approved designs and colors, that shown having three stripes, the middle one showing the natural wood and the outer stripes showing alternate blocks in the natural wood and color; the latter for the purposes of this illustration may be assumed to represent black ebony wood, and in practice would be done with a black stain or india ink.

25 In practice I use a transparent or translucent coating or filler on the bare wood to improve the ground coat 2, and also for the purpose of preventing the india ink and water colors from "running" between the grain of the wood, and thus guarding against ragged lines. This is especially important in using the india ink for outlining and striping. For this purpose I may use white shellac or dextrin applied as a thin coating on the wood by dipping or with a brush. After this coating is thoroughly dry I apply the ground coat 2, and proceed as above stated. The shellac or dextrin is not affected by the solution which I employ for softening the paint in working out the design. The shellac or dextrin coating is also useful in outlining the design before the ground coat 2 is applied, which in some cases may be desirable, and in some cases, owing to the nature of the design, necessary. When this is done, the entire design is worked out in india ink on the shellac or dextrin coating, omitting however the other color effects. After the design is thoroughly dry, the ground coat 2 is applied, but in this instance the coating must be of a color and density which will not obscure the design. After this coating is sufficiently dry the softening solution is applied with a brush following the outline of the design. The paint softening solution does not affect the india ink, hence when the softened paint is removed, the panel will appear as shown in the lower half of the drawing. Colors may now be applied, if desired, and then the finishing coat of varnish or other finish may be applied as above stated. In some cases, for instance where it is not desired to apply a filler to the wood before applying the ground coat, it is preferable to mix the dextrin with

the india ink or water colors to prevent "running." The dextrin solution is prepared by dissolving dextrin powder in warm water.

The paint softening solution which I employ contains oil of cloves, spirits of camphor, banana oil, castor oil and creosote in the following proportions: oil of cloves 75%—spirits of camphor 3%—banana oil 20%—castor oil 1% and creosote 1%. The effective constituent of this solution is oil of cloves and this oil may be used alone. As a substitute for oil of cloves I may employ bay oil or lemon oil, but I prefer oil of cloves for the reason that it gives sharper outlines to a design.

This solution may be applied in various ways, and for large designs a stencil may be employed, and instead of applying the solution with a brush, it may be sprayed on with a painter's air-brush. The solution acts also on varnish and when desired the surface to be decorated may be first coated with varnish, or my method may be employed to decorate panels, table-tops, and the like which already have a varnish finish.

My method may be employed to produce decorative effects on glass or other surfaces for various uses, and also for producing sign-boards on glass or similar surfaces. The procedure in all cases will be the same, except that when working on glassy surfaces the priming coat of shellac or dextrin will not be necessary and the outlining of the design may be done in any color or material capable of use directly on glass or on the ground coat 1. Therefore, all references in the specification and claims to the ornamentation of wood or panels for use in cabinet work, furniture, wall decorations, etc., are to be deemed to include glass, glassy or other surfaces or materials.

What I claim is:

1. A method of ornamenting wood, consisting in coating the surface with a coat of oil stain or paint of the desired color and allowing same to dry, then applying to the painted surface over the area of a desired design a solution containing an oil which softens the stain or paint, then removing the softened paint by rubbing with an absorbent material, and then applying one or more finishing coats of varnish or shellac.

2. A method of ornamenting wood, consisting in coating the surface with a coat of oil stain or paint of the desired color and allowing same to dry, then applying to the painted surface over the area of a desired design a solution containing an oil which softens the stain or paint, then removing the softened paint by rubbing with an absorbent material, then applying such additional colors upon the exposed surface as may be desired, and then applying one or more finishing coats of varnish or shellac.

3. A method of ornamenting wood, con-

- sisting in coating the surface with a coat of oil stain or paint of the desired color and allowing same to dry, then applying to the painted surface over the area of a desired 5 design a solution containing an oil which softens the stain or paint, then removing the softened paint by rubbing with an absorbent material, then outlining the design with india ink, and then applying one or 10 more finishing coats of varnish or shellac.
4. A method of ornamenting wood, consisting in coating the surface with a coat of oil stain or paint of the desired color and allowing same to dry, then applying to the 15 painted surface over the area of a desired design a solution containing an oil which softens the stain or paint, then removing the softened paint by rubbing with an absorbent material, then outlining the design with india 20 ink and applying such additional colors within the design as may be desired, and then applying one or more finishing coats of varnish or shellac.
5. A method of ornamenting wood, 25 consisting in coating the surface with a transparent coating, then applying a coat of oil stain or paint of the desired color and allowing same to dry, then applying to the painted surface over the area of a desired 30 design a solution containing an oil which softens the stain or paint, then removing the softened paint by rubbing with an absorbent material, and then applying one or more finishing coats of varnish or shellac.
- 35 6. A method of ornamenting wood, consisting in coating the surface with a transparent coating, then applying a coat of oil stain or paint of the desired color and allowing same to dry, then applying to the painted 40 surface over the area of a desired design a solution containing an oil which softens the stain or paint, then removing the softened paint by rubbing with an absorbent material, then outlining the design with india 45 ink and applying such additional colors within the design as may be desired, and then applying one or more finishing coats of varnish or shellac.
7. A method of ornamenting wood, 50 consisting in coating the surface with a coat of oil stain or paint of the desired color and allowing same to dry, then applying to the

painted surface over the area of a desired design a solution containing oil of cloves to soften the stain or paint, then removing the 55 softened paint by rubbing with an absorbent material, and then applying one or more finishing coats of varnish or shellac.

8. A method of ornamenting wood, consisting in coating the surface with a coat of oil stain or paint of the desired color and allowing same to dry, then applying to the painted surface over the area of a desired 60 design a solution containing oil of cloves to soften the stain or paint, then removing the 65 softened paint by rubbing with an absorbent material, then outlining the design with india ink and applying such additional colors within the design as may be desired, and then applying one or more finishing coats of 70 varnish or shellac.

9. A method of ornamenting wood, consisting in coating the surface with a transparent coating, then applying a coat of oil stain or paint of the desired color and allowing same to dry, then applying to the painted surface over the area of a desired design a solution containing oil of cloves to soften the stain or paint, then removing the 75 softened paint by rubbing with an absorbent material, then outlining the design with india ink and applying such additional colors within the design as may be desired, and then applying one or more finishing coats of varnish or shellac.

85 10. A method of ornamenting wood, consisting in coating the surface with dextrin, then applying a coat of oil stain or paint of the desired color and allowing same to dry, then applying to the painted surface over the area of a desired design a solution containing oil of cloves to soften the stain or paint, then removing the softened paint by rubbing with an absorbent material, then outlining the design with india ink on the 90 dextrin coating and applying such additional colors within the design as may be desired, and then applying one or more finishing coats of varnish or shellac.

This specification signed this 26th day of 100 July, 1926, at New York city, in the county and State of New York.

EDWARD FREUND.